

# UNITED STATES PATENT OFFICE.

GEORGE W. SARGENT, OF PITTSBURGH, AND JOSEPH W. WEITZENKORN, OF WASHINGTON, PENNSYLVANIA.

## ALLOY STEEL.

1,401,926.

Specification of Letters Patent. Patented Dec. 27, 1921.

No Drawing.

Application filed June 14, 1920. Serial No. 388,788.

To all whom it may concern:

Be it known that we, GEORGE W. SARGENT, a resident of Pittsburgh, in the county of Allegheny and State of Pennsylvania, and JOSEPH W. WEITZENKORN, a resident of Washington, in the county of Washington and State of Pennsylvania, have invented a new and useful Improvement in Alloy Steel, of which the following is a specification.

10 The object of the invention is to provide an improved manganese steel in which the desirable properties resulting from the use of manganese as a steel alloying element are increased and intensified, and in which 15 the undesirable effects of manganese are overcome or eliminated.

The steel alloy which we provide contains no more than about .80% carbon, from about 1.15% to 3% manganese, and from 20 a fraction of 1% to 1.25% molybdenum. The remainder of the alloy is iron with the exception of impurities, such as sulfur and phosphorus, which are usually found in 25 steels. While the invention contemplates alloy steels of the range of analysis just stated, the preferred steel contains from about .30% to .50% carbon, about 1.25% manganese and from about .25% to .75% molybdenum.

30 We have found that the addition to manganese steel of molybdenum in the proportions stated not only intensifies the physical properties of the steel, but also results in a steel having a wide range of hardening or 35 quenching temperature. With respect to the latter, the physical property curves of the present steel are of the same character as those shown in the Weitzenkorn Patent No. 1,287,153, in which the flattened curves

40 clearly illustrate the uniform physical properties of the steel when drawn within a wide range of temperatures. The steel is also much less sensitive than usual manganese steels to heating other than in drawing.

45 It has also been found that not only does the molybdenum itself become evenly distributed throughout the steel, but also that the molybdenum has the effect of similarly

distributing the manganese, with the result that piping and segregations are largely 50 eliminated, and the full benefit of all the alloying elements are realized.

The invention relates to alloy steels and has particularly to do with what are known as manganese steels.

55 Manganese is usually present in appreciable quantities in all ordinary carbon steels, chiefly as a result of the recarbonizing and deoxidizing of the steel by the use of ferro-manganese or spiegeleisen. However, unless a steel contains more than about 1% of manganese it is not usually regarded as manganese steel. When alloyed with 60 steel in a large enough percentage to be considered a characteristic alloying element, 65 manganese adds considerably to the tensile strength of the steel, but this advantage is usually accompanied by a loss in reduction of area and in elongation.

Manganese alloy steels containing not 70 more than about 1% carbon, and manganese not exceeding more than about 3% to 4% are pearlitic, and hence are similar in some respects to the well known pearlitic nickel steels. The general belief is that such steels 75 are brittle, but it has been found that the brittleness of pearlitic manganese steels is due largely to the failure or inability to heat treat them within the proper range of temperature. It has been found necessary to use great care 80 in heat treating such steels to develop the desired physical properties, because a relatively small divergence from the temperature which gives the desired property, results in a brittle condition. Due to this, as 85 well as to prolonged heating at temperatures above the critical range, and to too rapid cooling from such temperatures, the general belief is, as previously stated, that manganese steels are brittle.

90 While, as previously stated, the alloy may be used for any desired purpose, it is particularly suitable for case hardened articles. When a low carbon alloy of the character explained is case hardened, the case is of the 95 hard and tough austenitic condition com-

monly found in manganese high carbon steel, and the core is of very strong and tough pearlitic structure.

We claim:—

- 5 1. An alloy steel consisting of not more than .80% carbon, from about 1.15% to 3.00% manganese, from a fraction of 1% to about 1.25% molybdenum, and the remainder iron.
- 10 2. An alloy steel consisting of from about

.30% to .50% carbon, about 1.25% manganese, from about .25% to .75% molybdenum, and the remainder iron.

In testimony whereof, we have hereunto set our hands.

GEORGE W. SARGENT.

JOSEPH W. WEITZENKORN.

Witnesses:

MARX HERSCHE,

W.M. H. WEIS.